

# UNITED STATES PATENT OFFICE.

EDWARD GOLD, OF VANCOUVER, CANADA.

## METHOD OF PROTECTING PILES.

SPECIFICATION forming part of Letters Patent No. 686,282, dated November 12, 1901.

Application filed November 13, 1900. Serial No. 36,397. (No specimens.)

*To all whom it may concern:*

Be it known that I, EDWARD GOLD, a citizen of the United States, residing at Vancouver, in the Province of British Columbia and 5 Dominion of Canada, have invented a new and useful Process for Protecting Piles from *Teredo*, of which the following is a specification.

My invention is an improved process of 10 protecting piles and other timbers which are submerged or partly submerged in sea-water from the attacks of the *Teredo navalis*.

My improved composition consists of: slaked lime, two pounds; asphaltum, (commercial,) thirty pounds; cement, hydraulic, twenty-one pounds; brimstone, (crushed,) three pounds; crude creosote, one pound; asbestos, (powdered,) three pounds; sharp sand or granite rock crushed to a sufficient 20 degree of fineness, sixty pounds.

In the preparation of my improved composition the asphaltum and creosote are heated together in a suitable tank or vessel and well mixed by stirring. The slaked lime, cement, 25 brimstone, powdered asbestos, and sharp sand or powdered rock in about the proportions specified are first thoroughly mixed together while dry and then added to the melted asphaltum and creosote, the whole being thoroughly 30 mixed and forming a semifluid plastic mass.

In the application of my improved composition to a pile of other timber by my improved process I take a band or strip of fabric of suitable width and length and of porous and fibrous material and draw the same through the mass of the molten composition in the tank, so as to thoroughly coat and saturate said band, and the same while hot is 40 wrapped spirally around the pile where it is exposed to the action of the salt water and liable to the attack of the *teredo*, until a sufficient thickness is attained. This band may be of single thickness or may be double. 45 When doubled, the two thicknesses must be kept apart in the tank, so that the hot molten composition will not only saturate the material of the wrapper or band, but a considerable quantity of the composition will also be 50 inclosed between the two thicknesses thereof, and while the composition is still hot I apply an exterior coating of comminuted rock,

such as clean sand or crushed granite, heating the same to insure its embedding itself in and adhering firmly to the surface. By 55 thus immersing the fibrous material within the molten composition not only is the exterior surfaces thereof thoroughly coated therewith, but all strands and interstices thereof are charged and filled with the composition, 60 thereby rendering the same thoroughly waterproof and exceedingly tenacious in character. In some instances also I may further wrap a wire of galvanized iron around the outside, which embeds itself in the composition and 65 which strengthens and supports the compound; but usually this is not required, as the nature of my compound is strong and tough and not likely to splinter or break off. After the band has been wrapped around the 70 pile the composition in cooling sets and forms an extremely hard coating thereon, which will not melt or run under the heat of the sun, is not acted upon chemically by the salt water, is exceedingly tenacious, and is not 75 readily cracked or broken even when forcibly struck, as by a hammer.

My improved composition may be applied to form a coating of any desired thickness on the pile or other timber, and in practice the 80 same is applied of a thickness ranging from one-fourth to three-fourths of an inch.

My improved composition may be applied to a pile or other timber before shipment is made, as my composition is so hard and tenacious that piles or other timbers which have been coated therewith may be rafted or transported by rail or on shipboard and handled without unusual care without danger of injuring the composition thereon. 85

Having thus described my invention, I 90 claim—

1. The method of protecting piles and other timbers from the *Teredo navalis*, which consists in mixing asphaltum and creosote together in a heated condition, adding thereto a previously-admixed body of sand, cement, slaked lime, crushed brimstone and powdered asbestos, substantially in the proportions specified by weight, presenting thereby a semifluid mass, coating and saturating a suitable fabric with the composition while in a molten condition, and applying the said fabric while 95 hot to the surfaces of the piles or timbers to 100

be protected, substantially as and for the purpose specified.

2. The method of protecting piles and other timbers from the *Teredo navalis*, which consists in mixing creosote and asphaltum together in a heated condition, adding thereto a previously-admixed body of sand, cement, slaked lime, crushed brimstone and powdered asbestos, substantially in the proportions specified by weight, presenting thereby a semi-fluid mass, coating and saturating a suitable fabric with the composition while in a molten

condition, applying the said fabric while hot to the surfaces of the piles or timbers to be protected, and applying an exterior coating of heated comminuted rock to the fabric, substantially as described. 15

In testimony that I claim the foregoing as my own I have hereto affixed my signature in the presence of two witnesses.

EDWARD GOLD.

Witnesses:

W. A. CAMPBELL,  
H. G. MELLON.